

Jan. 8, 1929.

1,698,443

H. S. LUKENS ET AL

METHOD OF REMOVING COPPER OXIDE FROM COPPER

Filed March 31, 1924

2 Sheets-Sheet 1

*Fig. 1.*



*Fig. 2.*

CATHODES, ETC.

MELTING FURNACE

$Cu + Cu_2O$

DEOXIDIZING FURNACE

$Cu$

IMPURE COPPER

MELTING FURNACE

$Cu_2O + MeO$

SLAGGING FURNACE

$Cu$

*Fig. 3.*



MeO = OXIDE IMPURITY IN THE COPPER,  
XO = OXIDE CONSTITUENT OF THE SLAG.

WITNESS:

*Walter Schum*

INVENTORS:

*Russell P. Heuer*  
and *Hiram S. Lukens*.

BY

*Ed. Steele Jackson*  
ATTORNEY

Jan. 8, 1929.

1,698,443

H. S. LUKENS ET AL

METHOD OF REMOVING COPPER OXIDE FROM COPPER

Filed March 31, 1924

2 Sheets-Sheet 2



WITNESS:

*Walter Chiam*

INVENTORS:  
Russell P. Heuer  
and Hiram S. Lukens.  
BY  
*John Steele Jr.*  
ATTORNEY

Patented Jan. 8, 1929.

1,698,443

# UNITED STATES PATENT OFFICE.

HIRAM S. LUKENS AND RUSSELL P. HEUER, OF PHILADELPHIA, PENNSYLVANIA.

## METHOD OF REMOVING COPPER OXIDE FROM COPPER.

Application filed March 31, 1924. Serial No. 703,122.

Our invention relates to the deoxidation of copper.

Our main purpose is to deoxidize molten copper by slag and to use the slag over and over, reducing the oxide taken up by the slag either between the deoxidizing uses of the slag or preferably when circumstances permit continuously during the deoxidizing use of the slag.

10 A further purpose is to continuously deoxidize the slag during its use, either chemically or electrolytically, so as to maintain its effectiveness.

15 A further purpose is to pass molten copper intermittently or continuously through a bath in which its copper oxide is withdrawn by a slag.

20 A further purpose is to provide a slag above the molten metal and immiscible to the metal, into which the copper oxide within the metal may diffuse and in which the diffused copper oxide may be reduced chemically or electrically or otherwise to permit continued diffusion and extraction of 25 the copper oxide from the metal into the slag.

25 A further purpose, alternatively is to provide for intermittent or progressive removal of portions of the slag for treatment 30 to reduce its copper oxide content with corresponding substitution of fresh slag low in copper oxide for that removed.

35 A further purpose is to continuously take out copper oxide from a slag surmounting a bath of molten copper by electrolytic action.

40 A further purpose is to utilize a deoxidizing slag for deoxidizing a bath of molten metal at the same time that it is being treated by a reducing means, chemical or electrolytic, to prevent accumulation of oxide in the slag and to return to the bath the free metal of the oxide removed, preferably making the molten metal one of the electrolytic poles when the electrolytic 45 method is used.

45 Further purposes will appear in the specification and in the claims.

Our invention relates both to the methods or processes involved and to apparatus by 50 which these methods or processes may be carried out.

Figure 1 is a vertical section of diagrammatic apparatus using our invention.

55 Figures 2 and 3 show diagrammatically desirable arrangements of or schemes for operation, somewhat different in the two

figures to accommodate difference in the raw material requiring purification.

Figure 4 is a ternary diagram for the ternary system of copper, copper-oxide and a hypothetical slag, showing the tie-lines at one temperature.

Figures 5, 6, 7 and 8 are each representative of different experimental tests or series of tests, showing the experimentally determined tie-lines of the two liquid phases with different slags.

Commercial copper has been subject to the disadvantage of containing a small percentage of copper oxide in spite of many 70 efforts of different kinds to remove the copper oxide. This percentage in the best copper available has approximated  $\frac{1}{2}$  of 1%. Though small in quantity, this oxide has seriously affected the copper in altering its 75 physical properties and, more particularly, in increasing its electric resistance.

Efforts have been made to improve the copper by laboratory use of slags to remove the oxide of copper from the copper, but 80 this has never been capable of extensive use because of its laboratory character and primarily because the slags have never been freed from the absorbed copper oxide, the copper has not been improved greatly and 85 the operation has never been made a continuous one.

Electrolytic copper might at first glance seem to avoid this objection by being wholly free from copper oxide. However, it is not 90 possible to use the electrolytic copper in the form deposited without recasting. In this recasting process, copper oxide forms and dissolves within the molten copper. To correct this, carbon, hydrocarbons, etc., 95 have been introduced within and upon the molten copper, whereby the oxide content is reduced to about  $\frac{1}{2}$  of 1% copper oxide. This amount however remains in commercial copper and its ill-effect has been well 100 recognized. Efforts have been made to further remove it by carbon, hydro-carbons, etc., but if the reduction be continued the copper liberates a gas whilst cooling in the molds and the castings are unsuited for use. 105 These gases seem to gain access to the copper with the direct contact of copper and oxide reducing agents.

By our invention we deoxidize molten copper by floating upon its surface a suitable slag. Deoxidation results from the transfer of copper oxide to this slag. The 110

mechanism of such transfer is evident from consideration of the phase rule relations governing the distribution of one component, copper oxide between two liquid phases, 5 a slag-rich phase and a copper-rich phase.

When molten copper containing copper oxide comes into contact with an oxide-free slag the partial free energy of copper oxide in the copper is contrasted with the zero 10 partial free energy of copper oxide in the slag. Copper oxide moves into the slag from the copper to an extent determined by its partial free energies in the copper and in the slag, respectively, flow of copper oxide 15 from the copper into the slag ceasing when the rising partial free energy of copper oxide in the slag and the falling partial free energy of copper oxide in the copper reach the same level. At the same level of partial 20 free energy, different slags may have very different concentrations of copper oxide, which accounts for their corresponding different effectivenesses for the removal of copper oxide from the molten copper. Whatever 25 the slag there will at equilibrium be a definite concentration of copper-oxide in the slag for each concentration (no matter how small) in the copper, so that any one or many different slags may be used, but with 30 very different effectivenesses. We suggest a number which we have tried but without any thought that the list is complete nor that it includes all of the more highly effective slags.

35 In the slag deoxidation, to remove copper oxide so that the slag may be used again or may be used continuously, the slag is treated to remove copper-oxide. By electrolysis or other means the concentration of copper-oxide in the slag may be reduced practically 40 to zero, and it follows that the copper phase in equilibrium with such slag will approximate zero content of copper-oxide.

We remove the copper-oxide from the 45 molten copper by bringing the latter into contact with a slag and treat this slag to keep its copper-oxide content at or below a required amount.

While any slag which is effectively immiscible with molten copper and miscible with molten copper-oxide will serve the purpose, not all operative slags work equally well. Properties, melting-point, viscosity, vapor pressure, stability, etc., will favor certain slags. Other factors that may determine or affect the choice of a slag will be local conditions, rapidity and effectiveness in functioning and lack of corrosiveness to furnace linings.

50 The equilibrium distribution of copper oxide within the copper and within the slag will be better understood by a brief discussion of this subject from the standpoint of binary and ternary component relations between the molten two component system,

copper-oxide and copper, and the molten three component system copper-oxide, copper and slag, as follows:

Our slag deoxidation puts to useful application these phenomena which occur 70 when a molten, two-component system—copper and copper-oxide—is brought into contact with a third component—a slag, immiscible with molten copper and miscible with molten copper-oxide. The construction of a ternary diagram—Cu, Cu<sub>2</sub>O, slag—will show the resultant equilibria. 75

For a perfectly general treatment, we assume any slag, and develop the two binary equilibrium diagrams—Cu plus slag and 80 Cu<sub>2</sub>O plus slag—for temperatures exceeding the liquidus curves. To these can be added the binary diagram, Cu plus Cu<sub>2</sub>O, as determined by Slade and Farrow, (Proc. Roy. Soc'y, 1912, LXXXVII, page 524). 85

Since copper shows such limited liquid miscibility with both slag and oxide, most concentrations on the ternary diagram will show two liquids in equilibrium—one, in general, rich in slag, the other rich in copper; the total Cu<sub>2</sub>O present being divided between these two liquid phases. (See diagram, Figure 4.) 90

The composition of the liquid phase or phases present in the three-component system, copper, copper-oxide and slag, at a given temperature is graphically indicated in the ternary equilibrium diagram of Figure 4, which shows a diagram with a hypothetical slag miscible when molten with 100 molten copper-oxide and immiscible with molten copper. 95

This diagram shows that within the area abcd two immiscible liquids coexist for every ratio of the three components of the system. The composition of the one liquid (being molten slag containing dissolved copper oxide and some copper) will vary along dc with the simultaneous variation of the conjugate liquid (molten copper containing dissolved copper-oxide and, theoretically, some slag) along ab. For any given composition on ab (showing the copper-oxide content of the copper), only one composition on cd (showing the copper-oxide content of the 115 slag) can be maintained in equilibrium. The tie lines, such as fg, hj, etc., illustrate this relationship; compositions f and h of the impure copper require compositions g and j respectively of the impure slag. 120

We have experimentally determined the compositions of the co-existing liquids (impure copper and impure slag) for the lower portion of the ternary diagram for quite a number of different slags, with results that are plotted in Figures 5, 6, 7 and 8 with an assumption (substantially true) of negligible solution of slag into the copper and of negligible solution of copper into the slag. 125

These tie-lines are self-explanatory, the composition of the slag used being noted upon each tie-line. From these figures it will be noted that there is a wide divergence in the effectivenesses of the slags used. Among the better slags are seen to be the chlorides of calcium or barium mixed with a little sodium borate, and the chlorides of sodium or potassium mixed with a little sodium silicate, phosphate or borate. Sodium silicate alone and the chloride of potassium or sodium alone is seen to be less effective.

Figure 1 illustrates one of many arrangements for carrying out our process. Molten copper is introduced at 15 into the body 16 of the deoxidizing furnace 17. A trunnion and tilting mechanism is indicated diagrammatically for periodic pouring after the copper has been deoxidized or if desired the discharge may be by overflow (intermittent or continuous) at a spout 18. The refractory 19 seals the slag from the copper inlet and outlet and keeps the heat in the furnace. Above the slag which covers the molten copper may be advantageously floated a layer of carbon to help deoxidize the slag, or (and) a reducing gas or hydro-carbon might be introduced into the slag or above the slag as at 20, 20' respectively, for the same purpose. Liberated carbon monoxide or other gas effluent escapes from the furnace at 21.

Positive electrodes 24 and 25 are provided above the slag for electrolytic deposition of the copper of the  $Cu_2O$  diffused from the metal bath into the slag. The molten copper of the bath forms the negative electrode, electric connection being made from it, as indicated diagrammatically at 26, to the source of direct current, not shown.

Normally the electric resistance of the slag and carbon above the slag will be considerably less than the resistance of the slag proper, with the result that the slag-carbon mixture above the slag acts as a continuous positive electrode covering the whole slag bath. The electrolytic deposition of the copper is upon the copper of the bath. It will be obvious that the oxide of the slag is continuously reduced by both the electrolytic action of the current and by the carbon floating upon the slag and that if desired either may be used without the other.

If it be desired to supply additional heat to this reducing furnace, an alternating voltage may be impressed across the two carbon electrodes shown or across any other suitable electrodes (such as the pole pieces shown), the slag and metal bath being thereby used as a resistor for heating purposes.

Figure 2 indicates an advantageous scheme for carrying out our process when the raw material requiring purification is substantially free from other metals or metallic oxides than of copper. The raw material is

charged in the melting furnace, and the molten product containing copper oxide as impurity is delivered continuously or intermittently to the deoxidizing furnace which may advantageously be as shown in Figure 1. 70

It is quite desirable to perform the melting at sufficient distance from the deoxidizing furnace or container or under such conditions as to free the latter from the deteriorating effect upon the slag of the gases attending fuel combustion, so as to permit selection of slags independently of this factor and thus permit the use of cheap fuel heating. 75

If the raw material contain metallic impurities, these impurities may be removed in this process. Figure 3 illustrates a scheme of operation which accomplishes this. The slagging furnace shown receives molten metal with its impurities, from the melting furnace. If this metal be oxidized, oxides of the metallic impurities such as  $PbO$  accompany the copper oxide into the slag. It is to be noted, however, that the metals less noble than copper must be oxidized before any copper oxide will be present because the copper oxide would otherwise be decomposed to form the oxides of these other metals. This ordinarily becomes of little importance here because the other metals viewed as impurities are small in total quantity. 90

The impure slag is withdrawn continuously or intermittently and reduced in the separate reducing furnace to avoid contaminating the deoxidized metal with the reduction products of the slag. With strong reducing agents there may be slight disadvantageous reduction of a portion of the original slag. This is advantageously corrected by treating the reduction product from the reducing furnace with a suitable small portion of the unreduced slag which re-oxidizes the reduced portion of the slag for return with the slag product from the reducing furnace to the slagging furnace as indicated. 105

Obviously there may be a very wide variation in the details of our process according to the whim or particular need of the user and we claim all such in so far as they fall within the reasonable spirit and scope of our invention. 115

Having thus described our invention, what we claim as new and desire to secure by Letters Patent is:—

1. The process of freeing molten copper from the copper oxide dissolved in it, which consists in providing a medium into which the oxide will diffuse, taking up the oxide in the medium, removing the oxide from the absorbing medium and repeating the operation. 125

2. The process of freeing molten copper from the copper oxide dissolved in it, to purify the copper, which consists in remov- 130

- ing the oxide from the copper at the surface of the molten copper and returning the metal of the oxide to the surface of the copper while keeping the copper free from combination with the agent used in the removal.
3. The process of freeing molten copper from the copper oxide dissolved in it, to purify the copper, which consists in removing the oxide from the copper at the surface of the molten copper and concurrently returning the metal of the oxide to the surface of the copper while keeping the copper free from combination with the agent used in the removal.
- 15 4. In the art of removing copper oxide from molten copper by means of a slag, the invention which consists in slagging preliminarily melted copper with a material in which copper-oxide has low partial free energy as compared to its partial free energy in the same concentration in the molten copper, and treating the slag for use again.
- 25 5. In the art of removing copper oxide from molten copper by means of a slag, the step which consists in slagging the molten copper with a slag having lower partial free energy of copper oxide than the partial free energy of the copper oxide in the copper, and
- 30 30 treating the slag for use again.
6. The process of deoxidizing molten copper while keeping it free from added impurity which consists in covering the molten copper with slag capable of taking up copper oxide from the copper, taking up the copper oxide and treating the slag in place to reduce its copper oxide without adding any of the initial slag to the copper.
7. The process of treating molten copper to remove its copper oxide while keeping it free from added impurity which consists in treating the surface of the copper with slag, taking up the copper oxide while progressively deoxidizing the copper oxide in the slag and without adding any of the initial slag to the copper.
- 40 8. The process of deoxidizing molten copper continuously while keeping it free from added impurity, which consists in covering the molten copper with slag capable of taking up copper oxide from the copper and treating the slag in place as a continuing operation to reduce its copper oxide, the reduction of the copper oxide going on in the slag while the copper oxide is being extracted by the slag from the copper and without adding any of the initial slag to the copper.
- 50 9. The process of deoxidizing molten copper continuously while keeping it free from added impurity, which consists in covering the molten copper with slag capable of taking up copper oxide from the copper, taking up the copper oxide and reducing the copper oxide in the slag in position by a chemical reducing agent to maintain the effectiveness of the slag and without adding any of the initial slag to the copper.
10. The process of deoxidizing molten copper continuously keeping it free from added impurity which consists in covering the molten copper with slag capable of taking up copper oxide and chemically removing copper from the copper oxide content of the slag, as a continuing operation while it is taking up copper oxide from the copper and without adding any of the initial slag to the copper.
- 15 11. The process of deoxidizing molten copper continuously, which consists in covering the molten copper with slag capable of taking up copper oxide from the copper and electrolytically removing copper from the copper oxide in the slag and depositing it on the molten surface of the copper.
- 20 12. The process of deoxidizing molten copper continuously which consists in covering the molten copper with slag capable of taking up copper oxide and electrolytically removing copper from the copper oxide content of the slag, as a continuing operation while it is taking up copper oxide from the copper.
- 25 13. The process of deoxidizing copper by a slag having relatively high partial free energy as compared to the partial free energy of copper oxide in the same concentration in other slags at the same temperature, which consists in removing copper oxide from the slag while the slag is being used to slag the copper and thus keeping the copper oxide in the slag quantitatively so low as to permit continued diffusion of copper oxide from the copper into the slag.
- 30 14. The process of freeing molten copper from the copper oxide dissolved in it, which consists in providing a pool of molten copper, supplying molten copper with dissolved copper oxide in it to the pool at one point and withdrawing molten copper from the pool at another point while removing the oxide from the metal of the pool by diffusing the oxide into a slag and maintaining the absorbing capacity of the slag.
- 35 15. The process of freeing molten copper from the copper oxide dissolved in it, which consists in melting copper at one point, transferring it molten to another point where it is free from the conditions surrounding the melting and removing the oxide from the copper in the second position by diffusion into a slag which would be deteriorated by the gases attending fuel combustion.
- 40 16. The process of freeing molten copper from the copper oxide dissolved in it, which consists in melting copper at one point, transferring it molten to another point where it is free from the conditions surrounding the melting, removing the oxide from the

copper in the second position by diffusion into a slag which would be deteriorated by the gases attending fuel combustion and removing the molten purified copper.

5 17. The process of freeing molten copper from the copper oxide dissolved in it, which consists in melting copper at one point, transferring it molten to another point where it is free from the conditions surrounding the

melting, removing the oxide from the copper <sup>10</sup> in the second position by diffusion into a slag which would be deteriorated by the gases attending fuel combustion and reducing the copper oxide in the slag so as to permit use of the same slag over and over again.

HIRAM S. LUKENS.  
RUSSELL P. HEUER.